

Sept. 24, 1940.

A. SCHÖNHOLZER  
METHOD OF PRODUCING NONCURLING STIFFENED WOVEN  
FABRICS AND PRODUCT THEREOF  
Filed Dec. 6, 1937

2,215,938

Ordinary Organdie



FIG. 1.



FIG. 2.



FIG. 3.

Inventor:

Albert Schönholzer  
By Sommers & Young  
Attnys

## UNITED STATES PATENT OFFICE

2,215,938

METHOD OF PRODUCING NONCURLING  
STIFFENED WOVEN FABRICS AND PROD-  
UCT THEREOFAlbert Schönholzer, Horn, Switzerland, assignor  
to Raduner & Co., A.-G., Horn, SwitzerlandApplication December 6, 1937, Serial No. 178,446  
In Switzerland May 7, 1937

9 Claims. (Cl. 28—1)

This invention relates to noncurling stiffened woven fabrics.

It is known that all fabrics which have been subjected to stiffening treatment have a tendency towards curling, that is, rolling up especially at their edges. The degree of this tendency increases with the intensity of the application of the stiffening treatment. This tendency applies particularly to all fine fabrics of tightly twisted 5 yarns provided with permanent stiffeners, such as the typical stiffened, transparent fabrics, for instance, organdies made from muslin fabrics, and also voile-like fabrics which have been treated by swelling means to produce transparency and stiffness. This tendency toward curling is also present in heavier fabrics, for instance, double cloths, fabrics made in imitation of linen, etc., which have been treated to provide permanent stiffness. A further class of fabrics in which this tendency 10 toward curling is present is fabrics simply stiffened by plain sizing which may be or may not be fast to washing to some extent. The tendency towards curling is noticeable in such goods particularly during ironing, and hitherto this characteristic which is exceedingly annoying in working the goods could not be counteracted by any of the known finishing treatments.

Even measures, such as the known measure of calendering both faces of the fabric to the same 15 extent, are but temporarily effective, as their effect is in most cases destroyed by ordinary ironing, and is always wholly eliminated by washing and subsequent drying of the goods, so that these measures have been of no help to the user.

35 The extremely disadvantageous curling effect, particularly, when relatively fine muslin-like fabrics are involved, has been a great drawback to efforts to promote the more general use of such highly refined textile products.

40 An object of the present invention is to provide a method for completely eliminating the said extremely disadvantageous curling effect of fabrics, as experienced when spreading them out, or, even more, while cutting them to shape, particularly 45 under the influence of variations of atmospheric conditions as regards temperature or moisture content, and especially while ironing the fabrics.

In the accompanying drawing, Fig. 1 is an enlarged view of a face of an ordinary organdie fabric having all the yarns twisted in the same direction.

50 Fig. 2 is an enlarged view of a face of a fabric woven according to the present invention having the alternate yarns of the warp twisted opposite- 55 ly.

Fig. 3 is an enlarged face view of a fabric according to the present invention in which two threads of similar twist are alternated with two threads of opposite twist in both the warp and the weft.

5 According to the invention, fabrics are produced the warp or weft or both of which are woven by means of right and left hand twisted yarns interspersed therein, for instance, alternating individually or in groups, and are subjected to 10 the required refining treatments by means of any of the processes for producing transparency or other refining processes having a stiffening effect. It is to be understood that all methods hitherto used in the art for producing transparency by 15 swelling the fabric and which also produce stiffness either by means of acids or lyes or other swelling means as well as combinations of such methods are applicable for carrying out the invention.

20 The surprising result of numerous tests has shown that the solution of the problem of eliminating the curling of fabric, which problem has existed for a considerable number of years, is rendered possible by providing therein a compensating arrangement of right and left hand twisted 25 yarns. This compensating influence may be provided in either the warp or weft singly or in both conjointly, as desired. It may be provided by using threads having left hand and right hand twist 30 and arranging them alternately or in individual groups of threads of either kind of twisting, without the absolute necessity of interweaving exactly the same number of threads of each kind of twist, as considerable compensating influence is 35 obtained with a percentage of oppositely twisted yarns of much less than 50%. The percentage of oppositely twisted yarns required depends on the characteristics of the yarn employed. Provision may also be made for using such a group of op- 40 positely twisted yarns at the selvedge only but for practical purposes this measure is of minor importance, due to the fact that the selvedge is oftentimes cut off in working the cloth.

45 Furthermore, for the manufacture of fancy fabrics the provision of decorative stripes formed of oppositely twisted yarns so as to provide a fancy effect may suffice for obtaining the desired end, or yarns of unidirectional twist may be used for the individual fancy stripes together with an 50 arrangement of yarns twisted oppositely to each other in the ground fabric, or else all of the yarns of the ground fabric may be twisted oppositely to the direction of twist of the yarns of the stripes. As far as the broad principle of the in- 55

vention is concerned, it is immaterial in what manner the stiffening of the fabric, particularly the permanent stiffening thereof, is obtained, or what stiffening or swelling agents are used or 5 what concentrations, temperatures, durations of treatment are applied or whether the fabrics are subjected to any preliminary or after-treatments by means of which effects, such as, for example, pattern effects, crêpe or embossed effects or combinations of such are obtained.

According to the invention, provision is also made for eliminating the tendency towards curling from fabrics which have special effects, due to the use of special weaving methods, or to the 15 use of special refining treatments in connection with the employment of special yarns or to choice of other kinds of fibers therefor, or to varying of the preliminary treatment thereof, or due to printing influences and, which fabrics therefore, 20 have the tendency towards curling, by the use and arrangement of properly twisted interwoven yarns to exert a compensating influence on the otherwise curling fabric. It is to be understood that the term, yarn, in the present instance, is 25 intended to include single and inter-twisted yarns made from vegetable, animal or artificial fibers as well as from mixed fibers of any combination thereof, the fabric containing one or more different kinds of such yarns, as desired.

30 Broadly the use of oppositely twisted yarns in any feasible relative arrangements is admittedly a matter known per se for overtwisted, so-called crepe yarn fabrics the tension of the twist of which is relieved. Experience has shown that 35 crepe fabrics made of yarns twisted similarly but relieved from tension by shrinkage in the usual manner have no tendency towards curling, as the relief of tension stabilizes the yarns. But if the texture of a fabric made from unidirectionally 40 twisted crepe yarns were arbitrarily altered in an unnatural way by stretching and stiffening the fabric, the latter would then have a tendency to curl to a considerable extent. The invention is, therefore, not concerned with crepe fabrics which 45 have been treated in the usual way, or as this may be termed "creponised." The invention is, however, concerned with fabrics which are made from overtwisted yarns if these fabrics are provided with a plain stiffening effect.

50 There are further known fabrics in which, for example, the warp contains an alternate succession of yarns twisted in right hand and left hand direction for the purpose of obtaining a certain stripe effect which is brought about by the two 55 yarns reflecting the light in different manner. Such goods consist without exception in extremely soft, loose twist, fine fabrics, such as shirtings and fabrics which are used for making under-clothing, and do not curl even without the application of oppositely twisted yarns, on account of their softness.

In the following, a number of illustrative modes of procedure applicable for producing lasting or temporary stiffening effects according to the invention are mentioned by way of example only without limiting the invention to the same:

1. Modes of procedure for producing permanent stiffening effects by means of chemicals for swelling cellulosic or animal fibers, such as the 65 transparentizing and parchmentizing methods, i. e. treatment with acid, cuprammonium, zinc chloride, alkali lyes or the like.

2. Modes of procedures for producing semi-permanent stiffening effects, that is, effects 70 standing at least washing, by means of insoluble

sizing agents or such agents which are rendered insoluble, as cellulose solutions of any kind, glue, artificial resinous substances, lakes or the like in aqueous or non-aqueous solutions.

3. Modes of procedures for producing temporary stiffening effects, that is, effects which do not stand washing at all or only to a very limited extent, by means of any kinds of sizing agents of vegetable, animal or artificial nature.

The method according to the invention covers 10 also printing treatments for producing stiffening effects on fabrics which will have the tendency towards curling.

Apart from the plain transparent fabrics made from fine cotton fabric with which the invention 15 is concerned most of all, the invention is also of great importance for double cloths which are permanently stiffened so as to stand washing, for example, for use for collars or the like, and which, hitherto, could not be satisfactorily permanently stiffened, in general, due to their 20 annoying tendency towards curling.

According to the invention the crude fabric which is provided with the right and left hand twisted yarns may be subjected to other refining 25 treatments, i. e. it may be bleached, dyed, or printed, or the like either before, during or after the treatment which provides the stiffness.

As a particular example of the practice of the method according to the invention, a muslin fabric is woven of fine cotton yarns, for example a 30 80/120 fabric, that is, a fabric having its warp composed of count 80 yarns and its weft of count 120 yarns, and having a normal tight twist, for example, 32 turns per inch. The yarns employed 35 comprise a substantial proportion of both right hand and left hand twisted yarns, the said oppositely twisted yarns being alternated or at least mixed or interspersed substantially regularly throughout the fabric. The proportion of one type of yarn to the other type may be 50%. The fabric may then, if desired, be treated with known bleaching, dyeing, mercerising or printing processes. The thus prepared fabric is then subjected to an acid treatment of known character for producing stiffness and transparency, for example, treatment with sulfuric acid of a strength of 40 about 50-56° Bé., for a period of about 20 seconds at a temperature of about 15° C. The fabric is then neutralized, eventually mercerised and 45 washed. The resulting fabric is a permanently stiff, transparent organdie having no tendency to curl even after subsequent washing and during ironing. Voile fabrics also produced in this manner are also of importance.

55 It will be understood that the above specified conditions can be varied according to the circumstances and desired result in many respects that will occur to persons skilled in the art without departing from the spirit of the invention. In 60 place of the cotton yarns other cellulosic yarns as artificial silk, and linen, etc., may be employed. Also natural silk or wool are suitable. In place of the acid stiffening and transparentizing treatment other treatments such as alternate applications of caustic and acid may be employed to produce the stiffening. Also treatments with cuprammonium or zinc chloride may be substituted in known manner for the acid treatment to provide the stiffness. Additionally, when semi-permanent or temporary stiffness is desired, the hereinbefore mentioned treatments or applications of sizes may be substituted for the above-mentioned permanent stiffening treatments.

70 Various changes and modifications may be 75

made in the practice of my invention without departing from the principle or spirit thereof, by adding customary practice and established knowledge of the art to the present disclosure and the 5 scope of the appended claims is not to be regarded as limited except as specified therein.

What I claim is:

1. A thin, stiff, transparent, voile-like fabric substantially free of tendency to curl after hot ironing composed of substantial proportions of 10 both right hand and left hand twisted yarns, the oppositely twisted yarns being interspersed throughout the fabric with substantial regularity, the yarns being fine and tightly twisted and the 15 fabric being parchmentized.
2. A textile material comprising a thin, parchmentized, voile-like, stiff, open-mesh fabric composed of uniformly interspersed right-hand and left-hand twisted yarns, and having substantially 20 no tendency to curl after hot ironing.
3. A textile material comprising a parchmentized, stiff, transparent, open-mesh, voile fabric, composed of a substantial proportion of both 25 right-hand and left-hand, tightly twisted, fine, cotton yarns having about 32 turns per inch uniformly mixed in the fabric, and the fabric having substantially no tendency to curl after hot ironing.
4. The method of producing thin, stiff, open- 30 mesh, transparent fabrics having substantially no tendency to curl even during and immediately after hot ironing, comprising selecting tightly-twisted, fine yarns of natural cellulosic fibers of both left-hand and right-hand twist, weaving a 35 thin, open-mesh fabric of said yarns with the right- and left-hand twisted yarns substantially evenly distributed throughout, and parchmentizing said fabric to stiffen and transparentize the fabric.
5. A thin, stiff, textile fabric of parchmentized 40 muslin composed of both left- and right-hand tightly twisted, fine cotton yarns substantially uniformly distributed throughout the fabric, the fabric being relatively transparent and having an 45 open mesh and being substantially free of tendency to curl even after hot ironing.

6. A voile-like textile fabric which is open-meshed, thin, transparent and permanently stiff, composed of fine yarns of both right- and left-hand twist, said oppositely-twisted yarns being substantially uniformly distributed throughout 5 the fabric, said yarns having a tight twist of about 32 turns per inch and the fabric being parchmentized with retention of the tight twist, and said fabric having substantially no tendency to curl under the influence of hot ironing. 10

7. A permanently stiff, thin, transparent, open-mesh, muslin-type fabric, composed of fine yarns of both right- and left-hand twist, the yarns of said fabric being of about count 80 and count 120 in the warp and weft respectively, said oppositely-twisted yarns being substantially uniformly distributed throughout the fabric, said yarns having a tight twist of about 32 turns per inch and the fabric being parchmentized with retention of the 15 tight twist, and said fabric having substantially 20 no tendency to curl under the influence of hot ironing.

8. A voile-like textile fabric which is open-meshed, thin, transparent and permanently stiff, composed of fine yarns of both right- and left-hand twist, said oppositely-twisted yarns being substantially uniformly distributed throughout the warp of the fabric, said yarns having a tight 25 twist of about 32 turns per inch and the fabric being parchmentized with retention of the tight 30 twist, and said fabric having substantially no tendency to curl under the influence of hot ironing.

9. A voile-like textile fabric which is open-meshed, thin, transparent and permanently stiff, 35 composed of fine yarns of both right- and left-hand twist, said oppositely-twisted yarns being substantially uniformly distributed throughout the weft of the fabric, said yarns having a tight twist of about 32 turns per inch and the fabric 40 being parchmentized with retention of the tight twist, and said fabric having substantially no tendency to curl under the influence of hot ironing.

ALBERT SCHÖNHOLZER. 45